

## UNITED STATES PATENT OFFICE.

WILLIAM M. DEHN, OF SEATTLE, WASHINGTON.

## EXPLOSIVE AND PROCESS OF ITS MANUFACTURE.

No Drawing.

Application filed September 16, 1922. Serial No. 588,708.

To all whom it may concern:

Be it known that I, WILLIAM M. DEHN, a citizen of the United States, residing in Seattle, county of King, and State of Washington, have invented certain new and useful Improvements in Explosive and Processes of Its Manufacture, of which the following is a full, clear, and exact description.

This invention relates to the use of sodium nitrate in mixtures with the explosive composition manufactured by the process set forth in my application, Serial No. 462397, filed April 18, 1921, namely, the process of impregnating plant tissues with ammonium nitrate for explosive purposes. When comminuted sodium nitrate is incorporated with sawdust or other plant tissues which has been impregnated with ammonium nitrate, a new explosive composition is obtained that possesses the two useful qualities of low cost and effective blasting power. In other words, my invention is a composition of sodium nitrate, sawdust and ammonium nitrate; the sodium nitrate being distributed throughout the mass of ammonium nitrate which itself is present substantially intercellularly in respect to the plant tissue used. I have found that such distribution of materials in the composition is productive of an explosive which can advantageously be applied to certain kinds of blasting.

I have made experiments in impregnating comminuted plant tissues with sodium nitrate, similar to the experiments of impregnating plant tissues with ammonium nitrate, as set forth in my prior process. Though the compositions thus obtained possess the properties of sensitiveness of combustion and of potential power favorable for explosive use, they lack certainty of detonation, that is, the impregnated masses will burn without exploding, except when powerfully confined and detonated. It was observed that the sodium nitrate tended to melt and segregate in large masses, the explosive wave fell off rapidly, and the main charge usually continued merely to burn. However, when the finely divided sodium nitrate was properly incorporated with a sufficient quantity of a plant tissue impregnated with ammonium nitrate, the physical condition of minute separation thus secured in the composition prevented the deterrent effects of melting and segregat-

ing of the sodium nitrate and the whole composition was completely detonated by the usual blast-caps. The ammonium nitrate being distributed minutely and intimately, and during explosion yielding only gaseous products, serves as a leavening and vitalizing agent for the remainder of the composition.

It was found that the percentage of ammonium nitrate can be as low as 20% of the entire composition, but its best limits are above 30%.

In order to determine the favorable explosive limits of concentration of sodium nitrate with sawdust, the data of the following table were obtained. One gram charges of the explosives, prepared from fir sawdust, yielded the respective grams of sand crushed in the explosion bomb.

| Per cent of NaNO <sub>3</sub> | Mesh    | Sand | Per cent of NaNO <sub>3</sub> | Mesh    | Sand | 75   |
|-------------------------------|---------|------|-------------------------------|---------|------|------|
| A                             | 20-30   | 35.5 | 35                            | 100-200 | 21   |      |
|                               | 30-100  | 40.0 | 40                            | "       | 20   |      |
|                               | 100-200 | 50.0 | 45                            | "       | 34   |      |
| Impregnated average           |         | 41.8 | 50                            | "       | 39   |      |
| B                             | 20-30   | 23.5 | 55                            | "       | 45   | D 80 |
|                               | 30-100  | 30.0 | 60                            | "       | 48   |      |
|                               | 110-200 | 39.5 | 65                            | "       | 50   |      |
| Non-impreg. average           |         | 31.0 | 70                            | "       | 46   |      |
| C                             | 20-30   | 20.0 | 75                            | "       | 41   |      |
|                               | 100-200 | 44.0 | 80                            | "       | 32   |      |

It is observed in A that sawdust impregnated with sodium nitrate is superior to non-impregnated sawdust B and is also superior, potentially, to the best black gunpowders C. The most favorable concentration of sodium nitrate is 65%, as is shown in D, and this value lies about midway between the compositions necessary to yield CO and CO<sub>2</sub>, in accordance with the chemical equations:



Now, since the above data demonstrate that intimacy of contact of sodium nitrate in the impregnated sawdust is advantageous, it is evident that this intimacy may also be approximated in the use of sufficiently finely divided sodium nitrate, not impregnating the sawdust. Both of these compositions were, however, found to be so insensitive to detonation that they are of little or no practical use. But, when mixed with the cellulose-impregnated ammonium nitrate, they detonated easily and completely. Therefore, cellulose-impregnated ammonium nitrate serves as a detonating and sensitizing com-

ponent for mixture of sodium nitrate and cellulose, whether the latter are impregnated or not.

I have found that impregnation by water 5 solutions can be applied to plant tissues, ammonium nitrate and sodium nitrate in three ways so as to secure superior explosive properties over compositions of these same materials held in simple mingled mixtures. I 10 can impregnate the ammonium nitrate in a mass of plant tissues sufficient as the combustible for both of the nitrates and can finally add the powdered sodium nitrate. I can impregnate separate portions of the 15 plant tissues with the respective nitrates. I can impregnate simultaneously the entire mass of plant tissue with a solution of the two nitrates. The first of these three methods, impregnating the plant tissue with ammonium nitrate only, was found by experiment to be safer and more economical, since a smaller volume of water for impregnating is required and the hazards of spontaneous 20 inflammability with carbonaceous compositions of sodium nitrate are avoided.

Since my invention substantially comprises the process of sensitizing, within favorable explosive limits, finely divided sodium nitrate through the use of com- 30 minuted plant tissues impregnated with ammonium nitrate, it is clear that all three ways are within the scope of my claims, though I may prefer to use the first mentioned. When the first procedure is followed, sufficient plant tissues to supply the 35 combustion requirements of both nitrates must be employed. For examples, the table:

|                       | CO <sub>2</sub> |    |    |    | CO-CO <sub>2</sub> |    |    |    |
|-----------------------|-----------------|----|----|----|--------------------|----|----|----|
|                       | A               | B  | C  | D  | E                  | F  | G  | H  |
| Sawdust.....          | 17              | 19 | 21 | 23 | 23                 | 25 | 29 | 31 |
| Sodium nitrate.....   | 10              | 20 | 30 | 40 | 10                 | 20 | 30 | 40 |
| Ammonium nitrate..... | 73              | 61 | 49 | 37 | 67                 | 54 | 41 | 29 |

5 illustrates various percentages of the materials calculated to yield as explosion gases, respectively CO<sub>2</sub> and equimolecular quantities of CO and CO<sub>2</sub>. These mixtures represent varied costs of explosives resulting 0 therefrom and also varied explosive properties, such as sensitiveness, power, densities, rates and certainty of detonation. Practically, therefore, I use for my explosive 1.5 to 6 parts of sawdust impregnated with 5 3 to 7 parts of ammonium nitrate and mixed with 1 to 4 parts of powdered sodium nitrate.

The rates of detonation of this explosive can be varied by increasing the percentages 10 of sodium nitrate, so that such rates range all the way down from that of the prior composition, containing only plant tissue and ammonium nitrate, to ineffective non-detonating compositions containing a pre-ponderating percentage of sodium nitrate.

Rates of detonation can further be controlled by varying the densities through compression, or by employing different sizes of sawdust to be impregnated with ammonium nitrate.

The novelty of my invention resides in the processes of distribution of the components, so that they are brought into minute and intimate contact and so that, during detonation, the explosive wave can be carried 75 forward throughout the mass and substantially the full disruptive power can be obtained.

I claim:

1. The process of manufacturing an explosive composition of plant tissue, ammonium nitrate and an alkali metal nitrate, which comprises distributing the alkali metal nitrate in minute and intimate contact with sufficient plant tissue impregnated with ammonium nitrate.

2. The process of manufacturing an explosive composition of wood meal, ammonium nitrate and an alkali metal nitrate, which comprises distributing the alkali metal nitrate in minute and intimate contact with sufficient wood meal impregnated with ammonium nitrate.

3. The process of manufacturing an explosive composition of plant tissue, ammonium nitrate and sodium nitrate, which comprises distributing the sodium nitrate in minute and intimate contact with sufficient plant tissue impregnated with ammonium nitrate.

4. The process of manufacturing an explosive composition of wood meal, ammonium nitrate and sodium nitrate, which comprises distributing the sodium nitrate in minute and intimate contact with sufficient 105 wood meal impregnated with ammonium nitrate.

5. The process of manufacturing an explosive composition of plant tissue, ammonium nitrate and sodium nitrate, which comprises distributing powdered sodium nitrate throughout a mass of finely divided plant tissue impregnated with ammonium nitrate, the mass of plant tissue being sufficient to supply the combustion requirements of the 115 two nitrates.

6. The process of manufacturing an explosive composition of wood meal, ammonium nitrate and sodium nitrate, which comprises distributing powdered sodium nitrate throughout the mass of wood meal impregnated with ammonium nitrate, the mass of wood meal being sufficient for both nitrates.

7. The process of sensitizing the explosive 125 properties of mixtures of plant tissue and sodium nitrate which comprises bringing powdered sodium nitrate into minute and intimate contact with a quantity of com- minuted plant tissue impregnated with am-

- monia nitrate, the quantity of said plant tissue being sufficient for the combustion requirements, not only for the ammonium nitrate but also for the sodium nitrate.
- 5 8. The process of sensitizing the explosive properties of mixtures of wood meal and sodium nitrate which comprises bringing powdered sodium nitrate into minute and intimate contact with a quantity of wood
- 10 meal impregnated with ammonium nitrate, the quantity of said wood meal being sufficient for the combustion requirements not only for the ammonium nitrate but also for the sodium nitrate.
- 15 9. The process of manufacturing an explosive composition which comprises the intimate intermingling of 1-4 parts of powdered sodium nitrate with 1.5-6 parts of comminuted plant tissue impregnated with 3-7
- 20 parts of ammonium nitrate.
10. The process of manufacturing an explosive composition which comprises the intimate intermingling of 1-4 parts of powdered sodium nitrate with 1.5-6 parts of wood meal impregnated with 3-7 parts of ammonium nitrate.
11. The explosive comprising 1-4 parts of powdered sodium nitrate mechanically mixed with 1.5-6 parts of comminuted plant tissue impregnated with 3-7 parts of ammonium nitrate.
12. The explosive comprising 1-4 parts of powdered sodium nitrate mechanically mixed with 1.5-6 parts of wood meal impregnated with 3-7 parts of ammonium nitrate.

In testimony that I claim the foregoing, I hereto set my hand, this 25 day of August, 1922.

WILLIAM M. DEHN.